

1

3,362,780

PROCESS FOR DYEING TEXTILE MATERIALS  
 Robert Kuth, Cologne-Sulz, Otto Schneider, Cologne-Flittard, and Mathieu Quaedvlieg, Leverkusen, Germany, assignors to Farbenfabriken Bayer Aktiengesellschaft, Leverkusen, Germany, a German corporation  
 No Drawing, Filed Mar. 10, 1964, Ser. No. 350,685  
 Claims priority, application Germany, Mar. 16, 1963,

F 39,270

4 Claims. (Cl. 8—42)

The present invention relates to a process wherein textile materials are dyed in such a manner that the dyestuffs are padded or printed in the form of solutions or suspensions and subsequently fixed by heating; reference may be made, for example, to the Thermosol process described in "American Dyestuff Reporter," 1949, page 593. More particularly the present invention concerns a process wherein such a padding or printing of textile materials is carried out in the presence of water-soluble reaction products of aromatic, hydroaromatic or aliphatic mono- or poly-isocyanates with high-molecular hydroxy-alkylation products of compounds which contain at least 8 carbon atoms and possess only one single hydrogen atom capable of reacting with alkylene oxides.

The reaction products to be used according to the invention contain at least once the grouping



wherein R means an alkylene radical containing two to four carbon atoms, and X stands for the radical of a compound which contains at least 8 carbon atom and possesses only one single hydrogen atom capable of reacting with alkylene oxides, while n is a number between 20 and 200.

Suitable reaction products can be obtained, for example, by reacting at about 50–70° C. ethyl isocyanate, stearyl isocyanate, phenyl isocyanate, toluylene diisocyanate, hexamethylene diisocyanate, 1,4-diisocyanato-cyclohexane, 4,4'-diisocyanato-dicyclohexylmethane, 4,4'-diisocyanato-diphenylmethane,  $\omega,\omega'$  - diisocyanato-dimethylbenzene or 4,4',4"-triisocyanato-triphenylmethane with hydroxy-alkylation products which are prepared by the addition of alkylene oxides, such as ethylene oxide or propylene oxide, in a molecular ratio of 20–200:1, on monohydric alcohols or carboxylic acids containing at least 8 carbon atoms, such as especially lauryl alcohol, myristyl alcohol, palmityl alcohol, stearyl alcohol, oleyl alcohol, hydro-abetyl alcohol or lauric acid, myristic acid, palmitic acid, stearic acid, oleic acid, linoleic acid, abietic acid and naphthenic acids, furthermore isohexyl phenol, heptyl phenol, nonyl phenol, dodecyl phenol or dodecyl mercaptan as well as secondary monoamines, such as methyl stearyl amine.

The textile materials which are to be dyed or printed by the process according to the invention may be based on the most varied synthetic products, for example polyamides, such as polycaprolactam, polyadic acid, furamethylene diamide and polyamino-undecanic acid, furthermore polyurethanes or polyesters, such as those from terephthalic acid and ethylene glycol or 1,4-dimethylol cyclohexane, as well as especially polyacrylonitrile and copolymers of acrylonitrile with other vinyl compounds, for example acrylic acid esters, acrylic acid amides, vinyl-pyridine, vinyl chloride and vinylidene chloride. Furthermore, the process according to the present invention comprises the dyeing or printing of those textile materials which are produced from cellulose esters, for example from cellulose triacetate or butyrate. The process according to the present invention can also be applied to mixed fabrics of synthetic fibers or to mixed fabrics of synthetic

2

fibers with fibers of native origin, such as wool or cotton, for example.

As in the aforesaid known dyeing process, the greatest variety of dyestuffs can also be employed in the present case, for example dispersion dyestuffs, vat dyestuffs, acid wool dyestuffs, metal complex dyestuffs or basic dyestuffs. Mixed fabrics can be dyed, with a suitable choice of dyestuffs, according to a single or multiple bath process possibly with insertion of an exhaust process, or selectively, if desired.

It is also possible by the process according to the invention to dye synthetic fiber materials in a satisfactory manner with dyestuffs with which they could hitherto be dyed only according to the exhaust process or not at all. Thus, for example, it is now possible to dye or print polyamide fibers with 2:1-metal-chromium complex dyestuffs, or polyacrylonitrile fibers with dispersion dyestuffs.

The reaction products to be used according to the invention are in general employed in amounts of 0.1–10%, preferably in amounts of 0.2–5.0%, referred to the dye liquor or printing paste, in the form of solutions or dispersions; they may, however, also be admixed in suitable concentrations to the dyestuffs. If the reaction products are not sufficiently soluble from the start, nonionic emulsifiers, such as hydroxy-alkylation products of fatty alcohols, fatty acids, naphthenic acids, of abietic acid or polyaryl-, alkylaryl- and alkylphenols, as well as ionic emulsifiers such as alkylaryl or alkyl sulphonates, can be used as dispersing agents.

The reaction products to be employed according to the present invention ensure an even distribution of the dyestuffs before and after fixation; they prevent two-sidedness and selvedge runnings of the dyeings and impart a pleasant handle to the textile materials; moreover they substantially increase the dyestuff yield, render a satisfactory dyeing possible even when several dyestuffs are used and enable the fixation temperature to be kept lower by 10–20° C. or the duration of fixing correspondingly shorter than is customary with the Thermosol process mentioned in the beginning. In addition, the use of thickening agents otherwise necessary which may cause the machine aggregates to become sticky can be dispensed with.

If desired, other assistants may also be added to the dye liquors, e.g., softening agents, carriers, antistatic compounds and also hydrotopic agents for increasing the solubility of the dyestuffs.

As compared with the polyethers or amides which have already been proposed as auxiliary agents for the Thermosol process, for example in Belgian patent specifications Nos. 615,102 and 615,207, the reaction products to be used according to the present invention are distinguished by the fact that a still higher dyestuff yield can be achieved by their use.

The following examples serve to illustrate the invention without, however, limiting the scope thereof. The dyestuffs designated by (a) to (i) are specified in the list given at the end of the description.

60

EXAMPLE 1

A fabric of polyacrylonitrile threads is impregnated on the foulard with a liquor which contains per litre 20 g. of the dyestuff (a) and 20 g. of the product obtained by reaction of 1 mol of 2,4-toluylene diisocyanate with 1 mol each of the hydroxy-alkylation products which were produced by the addition of 180 mol of ethylene oxide on 1 mol of stearyl alcohol and by the addition of 170 mol of ethylene oxide on 1 mol of stearic acid. The fabric is then squeezed off to a weight increase of about 80% and dried at 80–140° C. The fabric is subsequently treated in a tenter frame at 180–195° C. for 45 seconds with hot air, then rinsed, washed and dried. The brilliant yellow dyeing

obtained on the fabric is distinguished by excellent levelness, a very high efficiency of the dyestuff and outstanding fastness.

When a liquor is employed which contains, instead of 20 g. of the polymethine dyestuff (a), 20 g. of the azo dyestuff (b) or 20 g. of the anthraquinone dyestuff (c), a red dyeing or a blue dyeing of similar properties is obtained.

#### EXAMPLE 2

A fabric of polycaprolactam is dyed, as described in Example 1, with a liquor which contains per litre 50 g. of the acid dyestuff (d) and, 20 g. of the product obtained by the reaction of 1 mol of 1,4-diisocyanato-cyclohexane with 1 mol each of the hydroxy-alkylation products prepared by the addition of 130 mol of ethylene oxide on 1 mol of stearyl alcohol and by the addition of 40 mol of ethylene oxide on 1 mol of abietic acid. With a high efficiency of the dyestuff a uniform blue dyeing is obtained.

#### EXAMPLE 3

Knitted material of polycaprolactam or nylon is dyed, as described in Example 1, with a liquor containing per litre 50 g. of the chromium complex of the dyestuff (e) and 20 g. of the product which was obtained by reacting at 70° C. 1 mol of 4,4'-diisocyanato-dicyclohexyl methane with 1 mol each of the hydroxy-alkylation products produced by the addition of 130 mol of ethylene oxide on 1 mol of oleyl alcohol and by the addition of 130 mol of ethylene oxide on 1 mol of oleic acid. The red dyeing obtained is distinguished by excellent general fastness properties. Dyeings of similar properties in yellow and blue shades are obtained by employing, instead of the dyestuff (e), the chromium complexes of the dyestuffs (f) or (g).

#### EXAMPLE 4

A fabric of polycaprolactam fibers is treated, as described in Example 1, with a liquor which contains per litre 40 g. of the dispersion dyestuff (h) and 10 g. of the product obtained by the reaction of 1 mol of 2,4-toluylene diisocyanate with 1 mol each of the hydroxy-alkylation products produced by the addition of 130 mol of ethylene oxide on 1 mol of nonylphenol and by the addition of 120 mol of ethylene oxide on 1 mol of lauric acid. A brilliant blue dyeing with good fastness properties and good levelness is obtained.

#### EXAMPLE 5

A fabric of polyethylene terephthalate fibers is dyed according to the instructions of Example 1 with a liquor which contains per litre 20 g. of the dyestuff (h) and 20 g. of one of the products obtained by the reaction of 1 mol of 2,4-toluylene diisocyanate with 1 or 2 mol of the hydroxy-alkylation product obtained by the addition of 130 mol of ethylene oxide on 1 mol of oleyl alcohol. A uniform blue dyeing is obtained with a dyestuff efficiency of more than 92%.

If, under otherwise equal conditions, the dispersion dyestuff (i) is employed instead of the dyestuff (h), then a red dyeing is obtained which is distinguished by a high levelness and fastness to sublimation.

#### List of dyestuffs

Designation: Explanation  
(a) ----- Dyestuff of German patent specification No. 666,081, Example 1.

- (b) ----- Quaternized dyestuff according to line 5 of the table of Example 6 of French patent specification No. 1,158,839.
- (c) ----- Azo dyestuff of German patent specification No. 1,011,396, Example 48.
- (d) ----- Dyestuff of German patent specification No. 933,353, 1st paragraph of Example 2.
- (e) ----- Azo dyestuff of French patent specification No. 1,058,651, Example 3.
- (f) ----- Azo dyestuff according to Colour Index, 2nd edition, No. 18690.
- (g) ----- Azo dyestuff of German patent specification No. 940,483, Example 6.
- (h) ----- Dyestuff of German patent specification No. 1,029,506, 1st paragraph of Example 1.
- (i) ----- Azo dyestuff 1-amino-2-cyano-4-nitrobenzene→N-bis-acetoxyethyl-aniline.

20 We claim:

1. In the process for the dyeing of textile materials of synthetic hydrophobic fibers, wherein the dyestuffs are padded or printed in the form of solutions or suspensions and subsequently fixed by dry heating, the improvement 25 whereby the padding or printing is carried out in the presence of a water-soluble reaction product of aromatic hydrocarbon, hydroaromatic hydrocarbon or alkylene mono- or polyisocyanates with high-molecular hydroxy-alkylation products of hydrocarbyl compounds which contain 30 at least 8 carbon atoms and possess only one single hydrogen atom capable of reacting with alkylene oxides, the resulting reaction product containing the radicals of the formula



35 wherein R is alkylene of 2-4 carbon atoms; X is an organic radical of the compounds which contain at least 8 carbon atoms; and n is an integer of 20-200.

2. The process of claim 1 wherein the dyeing step is effected with disperse dyes, acid dyes, basic dyes and 40 metalized azo dyes on hydrophobic synthetic polymeric fibers by dry heating.

3. The process of claim 1 wherein about .1-10% by weight of water soluble reaction product is utilized in the dyeing process.

45 4. The process of claim 3 wherein the reaction product is the product obtained by reacting

- (a) a first component selected from the group consisting of alkyl isocyanate, phenyl isocyanate, toluylene diisocyanate, hexamethylene diisocyanate, 1,4-diisocyanate-cyclohexane, 4,4'-diisocyanate-dicyclohexylmethane, 4,4'-diisocyanate diphenylmethane,  $\omega,\omega'$ -diisocyanate-dimethylbenzene and triisocyanate-tri-phenylmethane with
- (b) the reaction product of alkylene oxide with a monohydric alcohol, alkyl phenol, alkyl mercaptan or secondary monoamine effecting the reaction of (a) and (b) at a temperature of about 50-70° C.

#### References Cited

#### UNITED STATES PATENTS

2,085,706 6/1937 Schoeller et al. ----- 252-89  
3,288,551 11/1966 Raff ----- 8-21

60 65 J. TRAVIS BROWN, *Acting Primary Examiner.*  
DONALD LEVY, *Assistant Examiner.*